

1

2,930,670

### MOLTEN UREA DYEING PROCESS

Samuel Nelson Bradshaw, Coventry, and Harry B. Mann, Braintree, England, assignors to Courtaulds Limited, London, England, a British company

No Drawing. Application July 24, 1956

Serial No. 607,252

Claims priority, application Great Britain July 29, 1955

10 Claims. (Cl. 8—85)

This invention relates to the dyeing of textile materials. In the normal dyeing procedure textiles are treated with an aqueous solution or dispersion of a dyestuff at a temperature depending on the nature of the material being dyed and the materials are left in the dyebath for a considerable period and are then rinsed and dried. The dyebath may also contain one or more dyeing assistants, for example common salt or Glauber's salt or other compounds which assist the material in taking up the dye and give a uniform penetration of the material by the dye. In the normal dyeing process therefore, water is the usual medium in which the dye is transferred to the textile materials but in the specification of co-pending application U.S. Serial No. 428,375, filed May 7, 1954, and its continuation-in-part Serial No. 668,043, filed June 26, 1957, there is described a method of dyeing in which molten urea replaces water as the dyestuff transfer medium. In this method textile materials are treated with a dyestuff in the presence of urea and are maintained at a temperature between the melting point of urea and 160° C. Thus textile materials may be impregnated with an aqueous solution or dispersion of the dyestuff and the urea, the impregnated material is dried and then baked at a temperature above the melting point of the urea.

In any dyeing process, it is generally desirable for economic or other reasons to carry out the process at the lowest practicable temperature and accordingly, the object of the present invention is to modify the process of U.S. Serial No. 428,375 and its continuation-in-part Serial No. 668,043, filed June 26, 1957, to enable lower temperatures to be used.

According to the present invention textile materials are treated with a dyestuff in the presence of urea and one or more other substances soluble in urea and capable of lowering the melting point of the urea and are maintained at a temperature between the melting point of the mixture and 160° C.

The amount by which the melting point is lowered will depend on the nature and quantity of the substance or substances added. Any suitable substance (hereinafter referred to as a "melting point depressant" or "depressant") soluble in molten urea and capable of lowering its melting point may be used. These depressants may be used in amounts up to  $\frac{1}{3}$  of the weight of the urea, or up to their maximum solubility in urea if this is less than  $\frac{1}{3}$ . The following table gives examples of suitable substances together with their maximum solubility in urea and the amount required to lower the melting point by 10° C.

| Substance         | Maximum solubility (percentage by weight on weight of urea) | Percentage required (based on weight of urea) to lower melting point by 10° C. |
|-------------------|-------------------------------------------------------------|--------------------------------------------------------------------------------|
| Thiourea          | >33                                                         | 11                                                                             |
| Dicyandiamide     | >33                                                         | 11                                                                             |
| Boric acid        | >33                                                         | 10                                                                             |
| Glycerol          | >33                                                         | 12                                                                             |
| Ethylene glycol   | >33                                                         | 10                                                                             |
| Sodium chloride   | 25                                                          | 8                                                                              |
| Ammonium chloride | >35                                                         | 10                                                                             |
| Ammonium sulphate | 25                                                          | 25                                                                             |

2

Certain depressants, besides lowering the melting point of the urea, also have a beneficial effect in reducing the tendency of the urea to decompose at elevated temperatures. Examples of such substances are the ammonium salts of strong acids such as ammonium chloride and ammonium sulphate. The melting point depressants may also be decomposition products formed in situ by heating urea above its melting point and allowing it to resolidify. If heated for a sufficient time (for example from  $\frac{1}{2}$  to 2 hours) at a sufficiently high temperature (for example from 150° to 170° C.), the resolidified urea has a lower melting point than the pure urea and can be used in the process of the present invention. The following table shows the reduction in melting point obtained with different temperatures and times of heating.

| Temp., ° C. | Time (hours)                 | Melting point, ° C. |
|-------------|------------------------------|---------------------|
| 20          | (melting point of pure urea) | 132.7               |
| 150         | $\frac{1}{2}$                | 124                 |
| 150         | 1                            | 124                 |
| 160         | $\frac{1}{2}$                | 128                 |
| 160         | 1                            | 124                 |
| 170         | $\frac{1}{2}$                | 124                 |
| 25          | 170                          | 114                 |

The method of carrying out the present invention may be similar to that described in U.S. Serial No. 428,375 and its continuation-in-part Serial No. 668,043, filed June 26, 1957; thus the textile materials may be impregnated with an aqueous solution or dispersion of the urea and the melting point depressant and an aqueous solution or dispersion of the dyestuff or a single aqueous solution or dispersion of the dyestuff, the urea and the melting point depressant, dried, baked to effect the dyeing, washed to remove the urea and dried. The urea and the melting point depressant are preferably applied simultaneously from the same bath in an amount sufficient to give a take up of urea of 40 to 55 percent by weight of the dry textile material. The impregnation is preferably effected at room temperature. The time for the baking step will depend on the temperature used; in practice times varying from  $\frac{1}{2}$  to 15 minutes have been found adequate.

The process of the present invention is suitable for dyeing with dyestuffs which are soluble in molten urea for example direct cotton dyestuffs, dispersed acetate dyestuffs, soluble acetate dyestuffs, leuco esters of vat dyestuffs, aggregated acid dyestuffs and metal complex dyestuffs. It is particularly suitable for dyeing with direct cotton dyestuffs.

The process of the present invention is suitable for dyeing those textiles which are not deleteriously affected by the baking, for example textile materials of cotton, wool, regenerated cellulose, artificial protein fibres, cellulose esters, synthetic polyamides and synthetic polyesters and materials made from mixtures of two or more of these fibres. If the process is used for dyeing textiles from thermoplastic fibres having a comparatively low melting point for example certain vinyl resin fibres the baking should be carried out at the lowest temperature and for the shortest time permissible.

The textile materials may be dyed according to the process of the invention in any convenient form, for example, the process may be applied to woven or knitted fabrics or to threads, yarns or fibres.

Any suitable apparatus can be used to carry out the process; for example the textile material may be impregnated with the urea, the melting point depressant and a dyestuff from an aqueous solution on a pad mangle and the impregnated material may be dried and baked in an oven. The apparatus normally used for carrying out a

crease-resist treatment with a urea-formaldehyde resin on textile materials can be used without substantial alteration.

In the baking step in the process of the present invention the urea melts and acts as a dye transfer medium. The process of the present invention provides a simple and convenient alternative to the established practice of dyeing from aqueous dyebaths. The process is simple, quick, easy to control and eliminates many of the difficulties encountered in dyeing with aqueous dyebaths.

The process is particularly suitable for dyeing blends of two or more different fibres especially where one of the fibres shows a preferential absorption for the dyestuff from an aqueous dyebath, for example blends of viscose rayon fibres and regenerated protein fibres can be dyed in an even shade with a direct cotton dyestuff by the process of the present invention whereas the blends would be differentially dyed from an aqueous dyebath.

The invention is illustrated by the following examples in which the parts are by weight.

#### Example 1

A fabric woven from 100 percent viscose rayon staple yarn was padded at 100 percent expression through a solution at room temperature prepared as follows:

1 part of Durazol Yellow 3RS (I.C.I.)  
40 parts of urea  
5 parts of thiourea

were made up to 100 parts with water. The fabric was dried at 80°C. and then baked for 15 minutes at 130°C. The dyed sample was then washed for 10 minutes in cold water and dried at 80°C.

On subjecting the dyed fabric to the washing test as described in the Second Report of the Fastness Tests Committee of the Society of Dyers and Colourists (Journal of the Society of Dyers and Colourists, 1948, volume 64, pages 136-137, Test No. 1) it was found that the fabric dyed by the process of the present invention was of comparable fastness to a fabric dyed from a conventional aqueous dyebath.

#### Example 2

A fabric woven from 100 percent viscose rayon staple yarn was padded at 100 percent expression through a solution at room temperature prepared as follows:

1 part Durazol Rubine BS (I.C.I.) Color Index 28160  
40 parts of urea  
5 parts of boric acid

were made up to 100 parts with water. The fabric was dried at 80°C. and then baked for 15 minutes at 130°C. The sample was then washed, dried, and the dye fastness assessed according to the test described in Example 1. Very little dye was removed by this test.

#### Example 3

A fabric woven from continuous filament cellulose acetate yarn was padded at 65 percent expression through the following solution at room temperature:

3 parts of Duranol Violet 2R 300 (I.C.I.) Color Index 61100  
40 parts of urea  
5 parts of glycerol  
1 part of Dispersol VL (I.C.I.)

made up to 100 parts with water. The padded fabric was dried at 80°C. and then baked for 15 minutes at 125°C. The sample was then washed in cold water and dried at 80°C. On subjecting the dyed sample to the washing test described in Example 1 very little staining on the piece of undyed cellulose acetate was noted.

#### Example 4

A solution was prepared as follows:

1 part of Coomassie Violet 2R (I.C.I.) Color Index 45190  
5 40 parts urea  
5 parts sodium chloride

were made up to 100 parts with water.

A fabric woven from 100 percent continuous filament nylon yarn was padded through this solution at 60 percent expression and then dried at 80°C. The sample was then split into two equal parts, one only of which was then baked for 10 minutes at 130°C., washed in cold water and dried at 80°C.

Both samples were subjected to the washing test described in Example 1. The sample which had been baked showed satisfactory dye retention but much of the dye on the unbaked sample was removed during the washing test.

20

#### Example 5

A fabric woven from 100 percent regenerated protein staple yarn was padded at 100 percent expression through a solution prepared as follows:

25 1 part Carbolan Blue RS (J.S.D.C. 1947, p. 283) Color Index 62075  
40 parts urea  
5 parts ammonium chloride  
2 parts Calsolene Oil

30

were made up to 100 parts with water. The padded fabric was dried at 80°C. and then baked for 10 minutes at 125°C. The dyed fabric was finally washed in cold water and dried at 80°C. A sample subjected to the washing test described in Example 1 showed good dye retention, very little staining of the undyed fabric being noted.

40

#### Example 6

Some urea was heated at 160°C. until the melting point had fallen to 124°C. The melt of "cooked" urea was allowed to resolidify and then ground to a powder.

A solution was prepared as follows:

1 part of Durazol Yellow 3RS  
45 parts of "cooked" urea

were made up to 100 parts with water.

A fabric woven from 100 percent viscose rayon staple yarn was padded through this solution at 100 percent expression and dried at 80°C. The fabric was then baked for 15 minutes at 130°C., washed and redried.

On subjecting the dyed fabric to the wash test detailed in Example 1 there was very little bleeding of the dye onto the undyed fabric in the test.

55

What we claim is:

1. A process for dyeing organic textile materials which comprises impregnating the textile material with a solution of a mixture of urea and at least one another substance which is soluble in molten urea and capable of lowering the melting point of urea, the amount of said substance in the mixture being sufficient to lower the melting point of the urea by at least 10°C., and with an aqueous solution or dispersion of at least one dyestuff which is soluble in molten urea and is substantive to the textile material, drying the textile material at a temperature below the melting point of the mixture of urea and said substance, heating the dried material, in the absence of steam to a temperature between the melting point of the mixture of urea and said substance and 160°C. to melt the mixture whereby the urea in the mixture serves as a solvent for the dyestuff, from which solution transfer of the dyestuff to the material takes place, washing the dyed material to remove the urea and said substance and again drying the material.

70

2. A process as claimed in claim 1 wherein the textile

material is impregnated with a single solution of urea and the said substance in which the dyestuff is dissolved or dispersed.

3. A process as claimed in claim 1 wherein the textile material is impregnated with an aqueous solution of urea and the said substance.

4. A process as claimed in claim 1 wherein the substance used is thiourea.

5. A process as claimed in claim 1 wherein the substance used is boric acid.

6. A process as claimed in claim 1 wherein the substance used is glycerol.

7. A process as claimed in claim 1 wherein the substance used is sodium chloride.

8. A process as claimed in claim 1 wherein the substance used is ammonium chloride.

9. A process as claimed in claim 1 wherein the textile material is impregnated with urea in an amount suffi-

cient to give a take-up of urea of 40 to 55 percent by weight of the dry textile material.

10. A process as claimed in claim 9 wherein the amount of depressant is from about 8 to about 33 percent of the weight of the urea.

References Cited in the file of this patent

UNITED STATES PATENTS

|    |           |         |               |
|----|-----------|---------|---------------|
| 10 | 1,963,975 | Ellis   | June 26, 1934 |
|    | 2,080,254 | Dreyfus | May 11, 1937  |
|    | 2,564,225 | Mayers  | Aug. 14, 1951 |

FOREIGN PATENTS

|    |         |             |               |
|----|---------|-------------|---------------|
| 15 | 996,335 | France      | Aug. 29, 1951 |
|    | 230,891 | Switzerland | May 16, 1944  |

OTHER REFERENCES

Am. Dyestuff Report, p. 802, November 1950.